

# United States Patent Office

2.760.933

Patented Aug. 28, 1956

1

2,760,933

## LUBRICANTS

**Ellis K. Fields, Chicago, Ill., and Clyde S. Scanley, Ogden  
Dunes, Ind., assignors to Standard Oil Company, Chi-  
cago, Ill., a corporation of Indiana**

No Drawing. Application November 25, 1952,  
Serial No. 322,572

**20 Claims. (Cl. 252—32.7)**

This invention relates to improved compositions which are effective corrosion inhibitors and which are non-corrosive to silver, silver alloys and similar metal. More particularly, the invention pertains to lubricant compositions which are non-corrosive to such metals and inhibit the corrosion thereof by sulfur and/or corrosive sulfur-containing compounds.

Advances in the design and construction of internal combustion engines to produce improved and more efficient and economical engines have presented many problems in the lubrication of the modern internal combustion engine. To meet the increased severe demands upon engine lubricants, many types of lubricant additives have been developed to obtain certain desired characteristics thereof. Among the more effective addition agents which have been developed for compounding with lubricants are many sulfur-containing organic compounds, such as by way of example, sulfurized terpenes, sulfurized hydrocarbon oils, vegetable oils or animal oils, xanthate esters, organic polysulfides, particularly polyalkyl polysulfides, metal salts of organo-substituted thioacids of phosphorus, metal salts of the reaction products of a phosphorus sulfide and a hydrocarbon, such as for example, polybutenes and other polyolefins, and combinations of the foregoing.

Recent increased use of silver and similar metals in the construction of improved internal combustion engines has created new problems in the use of sulfur-containing additives in lubricants for such engines; the primary problem created being the corrosion of such silver parts of the engine by the sulfur-containing additives. While such corrosion can be eliminated by avoiding the use of sulfur-containing additives in lubricants for such engines, this solution of the problem is accompanied by the loss of the highly desired beneficial effects of the additives of this type.

It is an object of the present invention to provide a non-corrosive composition. Another object of the invention is to provide a composition non-corrosive to silver and similar metal. A still further object of the invention is to provide a composition which will inhibit the corrosion of silver and similar metal by sulfur and/or organo sulfur-containing compounds. A still further object of the invention is to provide a lubricant composition which is non-corrosive. Still another object of the invention is to provide a lubricant composition containing an addition agent which will inhibit the corrosion of silver and similar metal by sulfur and/or organo sulfur-containing compounds. A further object of the invention is to provide a method of inhibiting the corrosion of silver and similar metal. Still another object of the invention is to provide a method of lubricating internal combustion engines.

In accordance with the present invention the foregoing objects can be attained by incorporating in oleaginous compositions, particularly lubricant compositions, a small amount, namely from about 0.02% to about 15%, and preferably from about 0.5% to about 5%, of a carboxylic

24

ester of 2,5-dimercapto-1,3,4-thiadiazole having the general formula:



in which R and R' are hydrocarbon radicals, such as aliphatic, aryl and alkaryl radicals of from 2 to about 30 or more carbon atoms. Examples of suitable hydrocarbon radicals are butyl, hexyl, octyl, nonyl, decyl, dodecyl, tridecyl, hexadecyl, octadecyl, benzyl, butylphenyl, etc., radicals; R and R' can be the same or different radicals. These esters are readily prepared by reacting 2,5-dimercapto-1,3,4-thiadiazole with an organic acid chloride in the molar ratio of 1:2 at a temperature of from about 25° C. to about 130° C. for one-half to twenty hours. To facilitate the reaction, suitable solvents, for example, benzene or dioxane, can be used. The reaction product is freed of hydrogen chloride and any carboxylic acid by washing with a dilute aqueous alkali solution or by passing a benzene solution of the reaction products through a column of activated alumina.

Examples of carboxylic esters of 2,5-dimercapto-1,3,4-thiadiazole are:

25 Dilauroyl ester of 2,5-dimercapto-1,3,4-thiadiazole  
 Distearoyl ester of 2,5-dimercapto-1,3,4-thiadiazole  
 Dibehenoyl ester of 2,5-dimercapto-1,3,4-thiadiazole  
 Diarachidoyl ester of 2,5-dimercapto-1,3,4-thiadiazole  
 30 Dicaproyl ester of 2,5-dimercapto-1,3,4-thiadiazole  
 Lauroyl butyroyl ester of 2,5-dimercapto-1,3,4-thiadiazole  
 Ditridecyl ester of 2,5-dimercapto-1,3,4-thiadiazole  
 Lauroyl stearoyl ester of 2,5-dimercapto-1,3,4-thiadiazole  
 Di-p-t-butyl benzoyl ester of 2,5-dimercapto-1,3,4-thia-  
 35 diazole

The preparation of the herein-described esters is illustrated by the following examples:

### EXAMPLE I

40 A mixture of 87.2 grams (0.4 mole) lauroyl chloride, 30 grams (0.2 m.) 2,5-dimercapto-1,3,4-thiadiazole, and 50 cubic centimeters benzene was stirred and refluxed at 90° C. for fourteen hours, at which time there was substantially no further evolution of hydrogen chloride. The product, diluted with 300 cubic centimeters of benzene, was passed through a column of activated alumina and the filtrate evaporated on the steam bath. The recovered product, 104 grams, was a light brown solid having a melting point of 68-72° C. The product was the di-lauroyl ester of 2,5-dimercapto-1,3,4-thiadiazole, as indicated by the following analysis:

|                                              | C     | H    | N    |
|----------------------------------------------|-------|------|------|
| Calculated for $C_{26}H_{46}N_3S_3O_2$ ..... | 60.70 | 8.95 | 5.45 |
| Found.....                                   | 60.43 | 8.67 | 5.64 |

### EXAMPLE II

60 A mixture of 121 grams (.4 mole) commercial stearoyl chloride (containing some palmitoyl and oleyl chlorides), 30 grams (.2 mole) 2,5-dimercapto-1,3,4-thiadiazole and 100 cubic centimeters benzene was refluxed for sixteen hours. Two hundred grams benzene were then added and 65 the warm solution filtered through activated alumina and the diluent evaporated on a steam bath. 130 grams of a light brown semi-solid was obtained which had a sulfur content of 12.4% and a nitrogen content of 3.52%.

### EXAMPLE III

A mixture of 45 grams (.3 mole) 2,5-dimercapto-1,3,4-thiadiazole, 117.9 grams (.6 mole) p-t-butyl benzoyl

chloride and 100 cc. toluene was stirred at 110° C. for sixteen hours. 48 cc. pyridine was added, dropwise, the mixture stirred at 95° C. for three hours, cooled and filtered, and the filtrate stripped in vacuo. The semi-solid was dissolved in ether, the ether solution filtered and evaporated, leaving a solid residue which analyzed 8.7% S and 2.91% N.

The esters may also be prepared by reaction of the free carboxylic acids, acid anhydrides or acid esters with the 2,5-dimercapto-1,3,4-thiadiazole.

The above-described compounds are used in combination with lubricant base oils, such as hydrocarbon oils, synthetic hydrocarbon oils, such as those obtained by the polymerization of hydrocarbons, such as olefin polymers, for example, polybutenes, polypropylene and mixtures thereof, etc., synthetic lubricating oils of the alkylene-oxide type, for example, the "Ucon oils," marketed by Carbide and Carbon Corporation, as well as other synthetic oils, such as the polycarboxylic acid ester-type oils, such as the ester of adipic acid, sebacic acid, maleic acid, azelaic acid, etc.

While the above-described products can be suitably employed alone in concentrations of from about 0.02% to about 10%, preferably from about 0.25% to about 5%, in combination with a base oil, they are usually used in combination with other lubricant addition agents, which impart various desired characteristics to the base oil. Usually, these reaction products are used in conjunction with detergent-type additives, particularly those which contain sulfur or phosphorus and sulfur. Additives of this type are usually used in amounts of from about 0.002% to about 10%, and preferably from about 0.01% to about 5%. Among the phosphorus and sulfur-containing addition agents are the neutralized reaction products of a phosphorus sulfide and a hydrocarbon, an alcohol, a ketone, an amine or an ester. Of the phosphorus sulfide reaction product additives, we prefer to employ the neutralized reaction products of a phosphorus sulfide, such as a phosphorus pentasulfide, and a hydrocarbon of the type described in U. S. 2,316,082 issued to C. M. Loane et al., April 6, 1943. As taught in this patent, the preferred hydrocarbon constituent of the reaction is a mono-olefin hydrocarbon polymer resulting from the polymerization of low molecular weight mono-olefin hydrocarbons, such as propylene, butenes, amylenes, or copolymers thereof. Such polymers may be obtained by the polymerization of mono-olefins of less than 6 carbon atoms in the presence of a catalyst, such as sulfuric acid, phosphoric acid, boron fluoride, aluminum chloride, or other similar halide catalysts of the Friedel-Crafts type.

The polymers employed are preferably mono-olefin polymers or mixtures of mono-olefin polymers and isomono-olefin polymers having molecular weights ranging from about 150 to about 50,000 or more, and preferably from about 500 to about 10,000. Such polymers can be obtained, for example, by the polymerization in the liquid phase of a hydrocarbon mixture containing mono- and isomono-olefins, such as butylene and isobutylene at a temperature of from about -80° F. to about 100° F. in the presence of a metal halide catalyst of the Friedel-Crafts type, such as for example, boron fluoride, aluminum chloride, and the like. In the preparation of these polymers a hydrocarbon mixture containing isobutylene, butylenes and butanes recovered from petroleum gases, especially those gases produced in the cracking of petroleum oils in the manufacture of gasoline, can be used.

Another suitable polymer is that obtained by polymerizing in the liquid phase, a hydrocarbon mixture comprising substantially C<sub>8</sub> hydrocarbons in the presence of an aluminum chloride-complex catalyst. The catalyst is preferably prepared by heating aluminum chloride with iso-octane. The hydrocarbon mixture is introduced into the bottom of the reactor and passed upwardly through

the catalyst layer, while a temperature of from about 50° F. to about 110° F. is maintained in the reactor. The propane and other saturated gases pass through the catalyst, while the propylene is polymerized under these conditions. The propylene polymer can be fractionated to any desired molecular weight, preferably from about 500 to about 1000 or higher.

Other suitable polymers are those obtained by polymerizing a hydrocarbon mixture containing about 10% to about 25% isobutylene at a temperature of from about 0° F. to about 100° F., and preferably 0° F. to about 32° F. in the presence of boron fluoride. After the polymerization of the isobutylene together with a relatively minor amount of the normal olefins present, the reaction mass is neutralized, washed free of acidic substances and the unreacted hydrocarbons subsequently separated from the polymers by distillation. The polymer mixture so obtained, depending upon the temperature of reaction, varies in consistency from a light liquid to viscous oily material and contains polymers having molecular weights ranging from about 100 to about 2000, or higher. The polymers so obtained may be used as such, or the polymer may be fractionated under reduced pressure into fractions of increasing molecular weights and suitable fractions obtained reacted with the phosphorus sulfide to obtain the desired reaction products. The bottoms resulting from the fractionation of the polymer which may have Saybolt Universal viscosities at 210° F., ranging from about 50 seconds to about 10,000 seconds, are well suited for this purpose.

Essentially paraffinic hydrocarbons, such as bright stock residuums, lubricating oil distillates, petrolatums, or paraffin waxes, may be used. There can also be employed the condensation products of any of the foregoing hydrocarbons, usually through first halogenating the hydrocarbons with aromatic hydrocarbons in the presence of anhydrous inorganic halides, such as aluminum chloride, zinc chloride, boron fluoride, and the like.

Examples of other high molecular weight olefinic hydrocarbons which can be employed are cetene (C<sub>16</sub>), cerotene (C<sub>28</sub>), melene (C<sub>30</sub>), and mixed high molecular weight alkenes obtained by cracking petroleum oils.

Other preferred olefins suitable for the preparation of the phosphorus sulfide reaction products are olefins having at least 20 carbon atoms in the molecule of which from about 13 carbon atoms to about 18 carbon atoms, and preferably at least 15 carbon atoms are in a long chain. Such olefins can be obtained by the dehydrogenation of alkyl halides, preferably long chain alkyl halides, particularly halogenated paraffin waxes.

As a starting material there can be used the polymer or synthetic lubricating oil obtained by polymerizing unsaturated hydrocarbons resulting from the vapor phase cracking of paraffin waxes in the presence of aluminum chloride which is fully described in United States Patents Nos. 1,955,260, 1,970,402 and 2,091,398. Still another type of olefin polymer which may be employed is the polymer resulting from the treatment of vapor phase cracked gasoline and/or gasoline fractions with sulfuric acid or solid adsorbents, such as Fuller's earth, whereby unsaturated polymerized hydrocarbons are removed. The reaction products of the phosphorus sulfide and the polymers resulting from the volatilization of hydrocarbons as described for example in United States Patents Nos. 2,197,768 and 2,191,787 are also suitable.

Other hydrocarbons that can be reacted with a phosphorus sulfide are aromatic hydrocarbons, such as for example, benzene, naphthalene, toluene, xylene, diphenyl, and the like, or with an alkylated aromatic hydrocarbon, such as for example, benzene having an alkyl substituent having at least four carbon atoms, and preferably at least eight carbon atoms, such as a long chain paraffin wax.

The phosphorus sulfide-hydrocarbon reaction product can be readily obtained by reacting a phosphorus sulfide, for example, P<sub>2</sub>S<sub>5</sub>, with the hydrocarbon at a temperature

of from about 200° F. to about 500° F., and preferably from about 200° F. to about 400° F., using from about 1% to about 50%, and preferably from about 5% to about 25% of the phosphorus sulfide in the reaction. It is advantageous to maintain a non-oxidizing atmosphere, such as for example, an atmosphere of nitrogen above the reaction mixture. Usually, it is preferable to use an amount of the phosphorus sulfide that will completely react with the hydrocarbon so that no further purification becomes necessary; however, an excess amount of phosphorus sulfide can be used and separated from the product by filtration or by dilution with a hydrocarbon solvent, such as hexane, filtering and subsequently removing the solvent by suitable means, such as by distillation. If desired, the reaction product can be further treated with steam at an elevated temperature of from about 100° F. to about 600° F.

The phosphorus sulfide-hydrocarbon reaction product normally shows a titratable acidity which is neutralized by treatment with a basic reagent. The phosphorus sulfide-hydrocarbon reaction product when neutralized with a basic reagent containing a metal constituent, is characterized by the presence of retention of the metal constituent of the basic reagent.

The neutralized phosphorus sulfide-hydrocarbon reaction product can be obtained by treating the acidic reaction product with a suitable basic compound, such as hydroxide, carbonate, oxide or sulfide of an alkaline earth metal or an alkali metal, such as for example, potassium hydroxide, sodium hydroxide, sodium sulfide, calcium oxide, lime, barium hydroxide, barium oxide, etc. Other basic reagents can be used, such as for example, ammonia or an alkyl or aryl-substituted ammonia, such as amines. The neutralization of the phosphorus sulfide-hydrocarbon reaction product is carried out preferably in a non-oxidizing atmosphere by contacting the acidic reaction product either as such or dissolved in a suitable solvent, such as naphtha, with a solution of the basic agent. As an alternative method, the reaction product can be treated with solid alkaline compounds, such as KOH, NaOH, Na<sub>2</sub>CO<sub>3</sub>, K<sub>2</sub>CO<sub>3</sub>, CaO, BaO, Ba(OH)<sub>2</sub>, Na<sub>2</sub>S and the like at an elevated temperature of from about 100° to about 600° F. Neutralized reaction products containing a heavy metal constituent, such as for example, tin, titanium, aluminum, chromium, cobalt, zinc, iron and the like can be obtained by reacting a salt of the desired heavy metal with the phosphorus sulfide-hydrocarbon reaction product which has been treated with the phosphorus sulfide-hydrocarbon reaction product, which has been treated with a basic reagent, such as above described.

Other phosphorus sulfide reaction products which can be used are the reaction products of a phosphorus sulfide and a fatty acid ester of the type described in U. S. 2,399,243; the phosphorus sulfide-degras reaction products of U. S. 2,413,332; the reaction product of an alkylated phenol with the condensation product of P<sub>2</sub>S<sub>5</sub> and turpentine of U. S. 2,409,877 and U. S. 2,409,878; the reaction product of a phosphorus sulfide and stearonitrile of U. S. 2,416,807, etc.

The silver corrosion-inhibiting property of the above-described carboxylic esters of 2,5-dimercapto-1,3,4-thiadiazole is demonstrated by the data in Table I, which were obtained by subjecting mixtures of hydrocarbon oils, a neutralized reaction product of P<sub>2</sub>S<sub>5</sub> and a polybutene and carboxylic esters of 2,5-dimercapto-1,3,4-thiadiazole to the following test, hereinafter referred to as the modified EMD test:

A silver strip 2 cm. x 5.5 cm. with a small hole at one end for suspension, is lightly abraded with No. 0 steel wool, wiped free of any adhering steel wool, washed with carbon tetrachloride, air-dried and then weighed to 0.1 milligram. 300 cc. of the oil to be tested is placed in a 500 cc. lipless glass beaker, and the oil heated to a temperature of 300° F. (+2° F.) and the silver strip suspended in the oil so that the strip is completely immersed therein.

The oil in the beaker is stirred by means of a glass stirrer operating at 300 R. P. M. At the end of twenty-four hours, the silver strip is removed and while still hot rinsed thoroughly with carbon tetrachloride and air-dried. The appearance of the strip is then visually noted and given ratings according to the following scale:

- 10 1—Bright
- 2—Stained
- 3—Grey-Black
- 4—Black, Smooth
- 5—Black, Flake

15 After the visual inspection the silver strip is immersed in a 10% potassium cyanide solution at room temperature until the silver surface assumes its original bright or silver appearance. The silver strip is then washed successively with distilled water and acetone, air-dried and weighed.

20 The following lubricant compositions were subjected to the above test and the results obtained tabulated in Table I.

25 *Sample A.*—Control (solvent extracted SAE 30 oil + 3.3% barium-containing neutralized reaction product of P<sub>2</sub>S<sub>5</sub> and a polybutene of about 1000 molecular weight).

*Sample B.*—A + 0.75% ester of Example I.

*Sample C.*—A + 0.75% ester of Example II.

*Sample D.*—A + 0.75% ester of Example III.

Table I

| Sample: | Silver corrosion (wt. loss Mg) |
|---------|--------------------------------|
| A       | 20-25                          |
| B       | 0/1                            |
| C       | 0/1                            |
| D       | 0/1                            |

30 Since a weight loss of 20 milligrams is allowable, the ability of the 2,5-dimercapto-1,3,4-thiadiazole derivatives of this invention to inhibit silver corrosion is demonstrated by the above data.

40 The effectiveness of the herein-described esters of 2,5-dimercapto-1,3,4-thiadiazole in inhibiting corrosion of copper and/or lead-containing metals, such as for example, copper-lead alloys, is demonstrated by the data in Table II, obtained by subjecting lubricants containing the additive to the following test:

45 A copper-lead test specimen is lightly abraded with steel wool, washed with naphtha, dried and weighed to the nearest milligram. The cleaned copper-lead test specimen is suspended in a steel beaker, cleaned with a hot trisodium phosphate solution, rinsed with water, acetone and dried, and 250 grams of the oil to be tested, together with 0.625 grams lead oxide and 50 grams of 30-35 mesh sand charged to the beaker. The beaker is then placed in a bath or heating block and heated to a temperature of 300° F. (±2° F.) while the contents are stirred by means of a stirrer rotating at 750 R. P. M. The contents of the beaker are maintained at this temperature for twenty-four hours, after which the copper-lead test specimen is removed, rinsed with naphtha, dried and weighed. 50 The test specimen is then replaced in the beaker and an additional 0.375 grams of lead oxide added to the test oil. At the end of an additional twenty-four hours of test operation, the test specimen is again placed in the beaker together with an additional 0.250 gram of lead oxide and the test continued for another twenty-four hours (seventy-two hours total). At the conclusion of this time, the test specimen is removed from the beaker, rinsed in naphtha, and dried and weighed.

55 60 The loss in weight of the test specimen is recorded after each weighing.

65 65 This test, known as the sand stirring corrosion test, is referred to hereinafter as "SSCT."

70 75 The data obtained when subjecting Samples A and B above, to the foregoing test, are tabulated in Table II.



of a carboxylic ester of 2,5-dimercapto-1,3,4-thiadiazole having the general formula:



in which R and R' are hydrocarbon radicals.

11. A lubricant composition as described in claim 10 in which the phosphorus and sulfur-containing detergent-type lubricant additive is the neutralized reaction product of a phosphorus sulfide and a hydrocarbon. 10

12. A lubricant composition as described in claim 10 in which the phosphorus and sulfur-containing detergent-type lubricant additive is derived from an olefin polymer. 15

13. A lubricant composition as described in claim 10 in which the phosphorus and sulfur-containing detergent-type lubricant additive is a potassium-containing neutralized reaction product of a phosphorus sulfide and an olefin polymer. 15

14. A lubricant composition as described in claim 10 in which the phosphorus and sulfur-containing detergent-type lubricant additive is an alkaline earth-containing neutralized reaction product of a phosphorus sulfide and an olefin polymer. 20

15. A lubricant composition as described in claim 10 in which the phosphorus and sulfur-containing detergent-type lubricant additive is a barium-containing neutralized reaction product of a phosphorus sulfide and an olefin polymer. 25

16. A lubricant composition as described in claim 10, 30 in which the phosphorus and sulfur-containing detergent-type lubricant additive is a calcium-containing neutralized reaction product of a phosphorus sulfide and an olefin polymer.

17. A lubricant composition comprising a major propor- 35

tion of a hydrocarbon oil, from about 0.001% to about 10% of a neutralized reaction product of a phosphorus sulfide and an olefin polymer, from about 0.001% to about 10% of a sulfurized terpene normally corrosive to silver, and from about 0.02% to about 15% of a carboxylic ester of 2,5-dimercapto-1,3,4-thiadiazole having the general formula:



in which R and R' are hydrocarbon radicals.

18. A composition comprising a major proportion of a lubricating oil containing a compound, normally corrosive to silver, selected from elemental sulfur, a sulfur-containing organic compound and mixtures thereof and from about 0.02% to about 15% of dilauroyl ester of 2,5-dimercapto-1,3,4-thiadiazole.

19. A composition comprising a major proportion of a lubricating oil containing a compound, normally corrosive to silver, selected from elemental sulfur, a sulfur-containing organic compound and mixtures thereof and from about 0.02% to about 15% of distearoyl ester of 2,5-dimercapto-1,3,4-thiadiazole.

20. A composition comprising a major proportion of a lubricating oil containing a compound, normally corrosive to silver, selected from elemental sulfur, a sulfur-containing organic compound and mixtures thereof and from about 0.02% to about 15% of di-p-t-butyl benzoyl ester of 2,5-dimercapto-1,3,4-thiadiazole.

References Cited in the file of this patent

UNITED STATES PATENTS

2,690,999 Lowe et al. Oct. 15, 1954